

## UNITED STATES PATENT OFFICE

2,577,364

## RHODIUM PLATING

Frank Herbert Reid, Hounslow, England, assignor  
to The International Nickel Company Inc., New  
York, N. Y., a corporation of Delaware

No Drawing. Application August 18, 1948, Serial  
No. 44,978. In Great Britain August 19, 1947

5 Claims. (Cl. 204—47)

1

This invention relates to the electrodeposition of rhodium onto other metals and to solutions for use therein.

The electrodeposition of rhodium onto other metals for decorative or tarnish-resisting purposes is commonly effected with the use of electrolytes of the kind containing as the essential constituent rhodium sulphate or rhodium phosphate or a mixture of these two compounds together with varying proportions of free sulphuric acid or free phosphoric acid or a mixture thereof. The free acid is necessary to prevent hydrolysis of the rhodium compounds in the electrolyte with consequent precipitation of rhodium hydroxide.

I have found that electrolytes of this kind, when operated under normal plating conditions, tend to furnish rhodium deposits which become "milky" in appearance as the thickness increases. The exact thickness of the deposit at which the desired metallic brilliance is lost varies with the composition of the electrolyte and the operating conditions. Thus, deposits from phosphate electrolytes may become milky when they are only 2.5 millionths of an inch thick whereas deposits from phosphate-sulphate electrolytes may remain bright until they are as thick as 10 millionths of an inch. Deposits from sulphate electrolytes generally remain bright until they are about 5 to 7 millionths of an inch thick. Now the minimum thickness generally regarded as satisfactory in industrial practice is 5 millionths of an inch and it is desirable that the deposits should be two or three times as thick as this.

An object of this invention is to provide a rhodium-plating process by which light deposits thicker than the prior art deposits can be produced.

Another object of this invention is to produce improved rhodium deposits by means of a critical amount of phenol in the electrolyte.

A further object of the invention is to provide a novel phenol-containing electrolyte for use in rhodium plating.

I have discovered that if a critical amount of phenol (hydroxybenzene) is added to the electrolyte, the thickness of the rhodium deposits is greatly increased before their characteristic brilliance is lost or they become milky in appearance.

The phenol concentration lies within the range 0.07 to 0.5 gram per liter. At concentrations below the lower figure no significant improvement is obtained and at concentrations above the upper figure the deposits tend to be dark.

It is to be understood that bright deposits greater than 5 millionths of an inch thick and therefore utilisable for some purposes can be obtained with some electrolytes, particularly the phosphate-sulphate electrolytes, under suitable operating conditions, but even then the use of

2

phenol is advantageous because the deposits should as a general rule be thicker than the minimum and the risk of milkiness appearing before the desired thickness is reached can be eliminated. It is also to be understood that even with the use of phenol the deposits cease to be bright at thicknesses which vary with the composition of the electrolyte and the operating conditions.

In processes of the kind in question as carried on hitherto, it is usual to employ a rhodium concentration of 2 grams per liter of electrolyte, a current density of from 2 to 4 amperes per square decimeter and an operating temperature of from room temperature to about 60° C. but more usually from 35 to 45° C. In carrying out the present invention none of these figures is critical, but it is preferred to depart from the prior art practice only to the extent of adding the critical amount of phenol. Nevertheless, if desired the rhodium concentration may vary between, say, about 0.5 and about 5 grams per liter. The free acid must always be enough to prevent hydrolysis of rhodium compounds, as those skilled in the art will understand. Increase in the free acid content above, say, 20 milliliters of sulphuric acid per liter decreases the current efficiency and so is time-consuming and uneconomic. The current density must, of course, be high enough to ensure that the metal on which the deposit is being made will not be chemically attacked, but may be less than 2 amps./dm.<sup>2</sup>. High cathodic current densities, say above about 5 amps./dm.<sup>2</sup>, tend to cause deterioration of the electrolyte, so I prefer to avoid their use.

I have found that if the phenol concentration exceeds 0.3 gram per liter the thickness of the deposit before slight milkiness appears decreases when the lower temperatures are used. To obtain the best results at the higher concentrations, therefore, the higher temperatures should be used, e. g. at least 40° C. with a concentration as high as 0.4 gram of phenol per liter. The current efficiency falls off rapidly as the concentration of phenol increases, the reduction being more marked at room temperature than at higher temperatures, so the high temperatures are desirable for this reason. However, at the higher temperatures the electrolyte tends to deteriorate if the cathodic current density is high. For instance one electrolyte containing 0.2 gram of phenol per liter which had been furnishing bright deposits up to 60 millionths of an inch thick at room temperature and 40° C. using a current density of 4 amps./dm.<sup>2</sup> was subsequently electrolysed at a temperature of 60° C. with a current density of 10 amps./dm.<sup>2</sup> for 5 minutes and then gave deposits which were slightly milky when they were only 25 millionths of an inch thick. On being again electrolysed at 40° C. with a current density of 4 amps./dm.<sup>2</sup> it failed

to give deposits which remained bright up to 60 millionths of an inch thick, but rather the deposits were severely streaked and milky when they were about 30 millionths of an inch thick. To avoid this tendency it is desirable to maintain the current density in the normal range of from 2 to 4 amps./dm.<sup>2</sup>.

#### EXAMPLE I

An electrolyte of the phosphate-sulphate type was prepared by reducing five grams of insoluble rhodium chloride with hydrogen at a low temperature, extracting the residue of finely divided rhodium by heating with concentrated sulphuric acid, cooling, diluting, filtering and precipitating rhodium hydroxide from the cooled filtrate by neutralization with dilute ammonium hydroxide solution. The hydroxide was washed thoroughly, transferred to a beaker and stirred into a thin cream with water. Solution was readily effected on adding 5 mls. of 85% phosphoric acid and warming gently. The resulting solution was poured into a mixture of 17 mls. of concentrated sulphuric acid and 850 mls. of distilled water to produce an electrolyte containing per liter 2 grams of rhodium, 20 mls. of sulphuric acid and 5 mls. of phosphoric acid.

The electrolyte prepared as described was then used to deposit rhodium onto cathodes of polished nickel, and the results shown by Table I were obtained.

Table I

| No.    | Phenol concn. (gms./l.) | Current Density (amps./dm. <sup>2</sup> ) | Temp. (°C.) | Time (mins.) | Thickness of Rh (ins. $\times 10^{-6}$ ) | Appearance of deposit |
|--------|-------------------------|-------------------------------------------|-------------|--------------|------------------------------------------|-----------------------|
| 1..... | nil                     | 3                                         | 20          | 5            | 7                                        | Milky.                |
| 2..... | nil                     | 2                                         | 35          | 5            | 15                                       | Do.                   |
| 3..... | 0.07                    | 2                                         | 60          | 10           | 25                                       | Bright.               |
| 4..... | 0.07                    | 2                                         | 60          | 25           | 45                                       | Do.                   |

#### EXAMPLE II

An electrolyte of the sulphate type was prepared by diluting with water 25 mls. of a sulphate solution prepared as described in Example I to give a final composition as follows:

Rhodium (as sulphate) \_\_\_\_\_ grams/liter 2  
Free sulphuric acid \_\_\_\_\_ mls./liter 10

This electrolyte was also used for depositing rhodium onto nickel and the results shown in Table II were obtained.

Table II

| No.     | Phenol concn. (gms./l.) | Current Density (amps./dm. <sup>2</sup> ) | Temp. (°C.) | Time (mins.) | Thickness of Rh (ins. $\times 10^{-6}$ ) | Appearance of deposit |
|---------|-------------------------|-------------------------------------------|-------------|--------------|------------------------------------------|-----------------------|
| 5.....  | nil                     | 2                                         | 20          | 6            | 10                                       | Milky.                |
| 6.....  | nil                     | 2                                         | 40          | 1.5          | 10                                       | Do.                   |
| 7.....  | nil                     | 2                                         | 60          | 1.5          | 6                                        | Do.                   |
| 8.....  | nil                     | 4                                         | 20          | 4.2          | 14                                       | Do.                   |
| 9.....  | nil                     | 4                                         | 40          | 1.75         | 7                                        | Do.                   |
| 10..... | nil                     | 4                                         | 60          | 2.1          | 14                                       | Do.                   |
| 11..... | 0.2                     | 4                                         | 20          | 60           | 131                                      | Bright.               |
| 12..... | 0.2                     | 4                                         | 60          | 10           | 52                                       | Do.                   |
| 13..... | 0.2                     | 4                                         | 60          | 5            | 37                                       | Do.                   |
| 14..... | 0.2                     | 4                                         | 60          | 6            | 28                                       | Do.                   |

The concentrations of phenol quoted above are illustrative and may be varied under appropriate operating conditions and still give satisfactory plating. The effect of variation in the phenol content is shown by the following example.

#### EXAMPLE III

A sulphate electrolyte containing per liter 2 grams of rhodium and 10 mls. of sulphuric acid gave the results shown in Table III when electrolysed at a current density of 4 amps./dm.<sup>2</sup>.

Table III

| No.     | Phenol concn. (gms./l.) | Temp. (°C.) | Time (mins.) | Thickness of Rh (ins. $\times 10^{-6}$ ) | Appearance of deposit |
|---------|-------------------------|-------------|--------------|------------------------------------------|-----------------------|
| 15..... | 0.1                     | 60          | 5            | 27                                       | Bright.               |
| 16..... | 0.3                     | 60          | 12           | 79                                       | Do.                   |
| 17..... | 0.4                     | 60          | 21           | 118                                      | Do.                   |
| 18..... | 0.5                     | 60          | 17           | 101                                      | Do.                   |

#### EXAMPLE IV

A phosphate electrolyte was made by dissolving rhodium hydroxide in phosphoric acid and diluting the phosphate solution to give a concentration, per liter, of 2 grams of rhodium and 20 mls. of phosphoric acid. On electrolysing this solution with a current density of 4 amps./dm.<sup>2</sup> the results shown in Table IV were obtained.

Table IV

| No.     | Phenol concn. (gms./l.) | Current Density (amps./dm. <sup>2</sup> ) | Temp. (°C.) | Time (mins.) | Thickness of Rh (ins. $\times 10^{-6}$ ) | Appearance of deposit |
|---------|-------------------------|-------------------------------------------|-------------|--------------|------------------------------------------|-----------------------|
| 19..... | nil                     | 4                                         | 20          | 2            | 2.5                                      | Slightly milky.       |
| 20..... | 0.1                     | 4                                         | 20          | 10           | 15                                       | Bright.               |

The metals onto which rhodium may be plated according to the invention are any that are compatible with the acid electrolytes and include, besides nickel, nickel silver, gold, platinum, palladium, copper and brass.

I claim:

1. In the process for electro-depositing thick plates of bright rhodium on metal using aqueous, acid electrolyte containing at least one rhodium compound from the group consisting of rhodium phosphate and rhodium sulfate in an amount sufficient to provide said electrolyte with about 0.5 to about 5 grams per liter of rhodium, and free acid from the group consisting of phosphoric acid and sulfuric acid in an amount sufficient to prevent hydrolysis of the rhodium compound but not exceeding about 20 milliliters per liter of electrolyte; the improvement which comprises incorporating in said electrolyte about 0.07 to about 0.5 gram per liter of phenol whereby thick, light-colored and bright rhodium electro-deposits are obtained at thicknesses of at least about 10 millionths of an inch on metal surfaces by employing the aforesaid phenol-containing acid electrolyte.

2. In the process for electro-depositing thick plates of bright rhodium on metal using aqueous, acid electrolyte containing at least one rhodium compound from the group consisting of rhodium phosphate and rhodium sulfate in an amount sufficient to provide said electrolyte with about 2 grams per liter of rhodium, and free acid from the group consisting of phosphoric acid and sulfuric acid in an amount sufficient to prevent hydrolysis of the rhodium compound but not exceeding about 20 milliliters per liter of electrolyte; the improvement which comprises incorporating in said electrolyte about 0.07 to about 0.5 gram per liter of phenol whereby thick, light-colored and bright rhodium electro-deposits are

obtained at thicknesses of at least about 10 millionths of an inch on metal surfaces by employing the aforesaid phenol-containing acid electrolyte.

3. A process for the production of thick, bright electro-deposits of rhodium on metal which comprises establishing a rhodium-plating electrolyte containing about 0.5 to about 5 grams per liter of rhodium provided by at least one rhodium compound from the group consisting of rhodium phosphate and rhodium sulfate, acid from the group consisting of phosphoric acid and sulfuric acid in an amount sufficient to prevent hydrolysis of the rhodium but not exceeding more than about 20 milliliters of acid per liter of electrolyte, about 0.07 to about 0.5 gram per liter of phenol; and electrolytically depositing rhodium from said electrolyte onto said metal at a current density between about 2 and about 4 amperes per square decimeter and at a temperature between about room temperature and about 60° C. to produce thick, light-colored and bright rhodium electro-deposits at thicknesses of at least about 10 millionths of an inch on said metal immersed as cathode in said electrolyte.

4. An electrolyte for use in obtaining thick electro-deposits of bright rhodium on metal which comprises an aqueous, acid bath containing about 0.5 to about 5 grams per liter of rhodium provided by at least one rhodium compound from the group consisting of rhodium phosphate and rhodium sulfate, acid from the group consisting of phosphoric acid and sulfuric acid in an amount sufficient to prevent hydrolysis of the rhodium but not exceeding about 20 milliliters of acid per liter of electrolyte, and about 0.07 to about 0.5 gram per liter of phenol whereby thick, light-colored and bright rhodium electro-deposits at thicknesses of at least about 10 millionths of an inch can be obtained on metal surfaces when employing the aforesaid phenol-containing, aque-

ous, acid electrolyte in electro-depositing rhodium onto metal surfaces.

5. An electrolyte for use in obtaining thick electro-deposits of bright rhodium on metal which comprises an aqueous, acid bath containing about 2 grams per liter of rhodium provided by at least one rhodium compound from the group consisting of rhodium phosphate and rhodium sulfate, acid from the group consisting of phosphoric acid and sulfuric acid in an amount sufficient to prevent hydrolysis of the rhodium but not exceeding about 20 milliliters of acid per liter of electrolyte, and about 0.07 to about 0.5 gram per liter of phenol whereby thick, light-colored and bright rhodium electro-deposits at thicknesses of at least about 10 millionths of an inch can be obtained on metal surfaces when employing the aforesaid phenol-containing, aqueous, acid electrolyte in electro-depositing rhodium onto metal surfaces.

FRANK HERBERT REID.

#### REFERENCES CITED

The following references are of record in the file of this patent:

#### UNITED STATES PATENTS

| Number    | Name             | Date          |
|-----------|------------------|---------------|
| 1,895,675 | Mathers          | Jan. 31, 1933 |
| 1,981,820 | Zimmerman et al. | Nov. 20, 1934 |
| 2,078,014 | Oplinger et al.  | Apr. 20, 1937 |
| 2,119,304 | Viers et al.     | May 31, 1938  |
| 2,250,556 | Stareck          | July 29, 1941 |

#### FOREIGN PATENTS

| Number  | Country       | Date          |
|---------|---------------|---------------|
| 446,393 | Great Britain | Apr. 29, 1936 |

#### OTHER REFERENCES

40 Transactions of the Electrochemical Society, vol. 80 (1941), pp. 494 to 497.